# EUROPEAN PATENT SPECIFICATION

(11) **EP 2 160 453 B1**
(45) Date of publication and mention of the grant of the patent: **11.07.2012**
(21) Application number: 08755495.2
(22) Date of filing: 15.05.2008
(51) Int. Cl.: C10M 141/06, C10M 129/76

(54) **LUBRICATING COMPOSITION CONTAINING SUPHUR, PHOSPHOROUS AND ASHFREE ANTIWEAR AGENT BASED ON A CITRIC ACID DERIVATIVE AND AMINE CONTAINING FRICTION MODIFIER**
SCHMIERMITTELZUSAMMENSETZUNG, ENTHALTEND SCHWEFEL-, PHOSPHOR- UND ASCHEFREIES ANTIVERSCHLEISSMITTEL AUF BASIS EINES ZITRONENSÄUREDERIVATS UND AMINHALTIGEN REIBUNGSMODIFIKATOR
COMPOSITION LUBRIFIANTE CONTENANT UN AGENT ANTI-USURE SANS CENDRES, SANS SOUFRE ET SANS PHOSPHORE À BASE D'UN DÉRIVÉ D'ACIDE CITRIQUE ET UN AGENT DE MODIFICATION DU FROTTEMENT CONTENANT UNE AMINE

(30) Priority: 24.05.2007 US 939952 P
(43) Date of publication of application: 10.03.2010
(73) Proprietor: The Lubrizol Corporation, Wickliffe OH 44092-2298 (US)
(72) Inventor: KOCSIS, Jody, Wickliffe, Ohio 44092-2298 (US); MOSIER, Patrick E., Wickliffe, Ohio 44092-2298 (US)
(74) Representative: Mallalieu, Catherine Louise
(86) International application number: PCT/US2008/063653
(87) International publication number: WO 2008/147700

(56) References cited:
- EP-A- 0 721 978
- WO-A-2006/044411

## Description

### FIELD OF INVENTION

The invention provides a lubricating composition containing an oil of lubricating viscosity, an amine-containing friction modifier, and an ashless antiwear agent. The lubricating composition is suitable for lubricating an internal combustion engine.

### BACKGROUND OF THE INVENTION

Engine manufacturers have focused on improving engine design in order to improve fuel economy and efficiency (typically, based on Federal Corporate Average Fuel Economy (CAFE) standards). Whilst improvements in engine design and operation have contributed, improved formulation of engine oil lubricant may also improve fuel economy and efficiency. Lubricants function to reduce and disperse engine deposits which accumulate when the engines are running. They also serve to reduce the friction between sliding moving parts (typically metallic or ceramic) that are in contact.

It is well known for lubricating oils to contain a number of additives used to protect the mechanical devices such as internal combustion engines from wear, soot deposits and acidity build up. A common antiwear additive for engine lubricating oils is zinc dialkyldithiophosphate (ZDDP). It is believed that ZDDP antiwear additives protect the engine by forming a protective film on metal surfaces. ZDDP is also believed to have a detrimental impact on fuel economy and efficiency. Consequently, engine lubricants also contain friction modifier to obviate the detrimental impact of ZDDP on fuel economy and efficiency. Both ZDDP and friction modifier function by adsorption on sliding surfaces, and each may interfere with each other's respective functions.

Further, engine lubricants containing phosphorus compounds and sulphur have been shown to contribute in part to particulate emissions, and emissions of other pollutants. In addition, sulphur and phosphorus tend to poison the catalysts used in catalytic converters, resulting in a reduction in performance of said catalysts.

With increasing control of emissions (often associated with contributing to NOₓ formation, SOₓ formation, formation of sulphated ash and reducing the efficiency of after-treatment catalytic converters) there is a desire towards reduced amounts of sulphur, phosphorus and sulphated ash in engine oils. However, reducing the levels of antiwear additives such as ZDDP, is likely to increase wear and result in other detrimental performance of an engine.

Whilst the presence of ZDDP reduces wear, and reduced amounts of ZDDP reduce emissions, engines experience corrosion. Corrosion of engine components containing metals such as copper or lead is known. However, many known corrosion inhibitors interact with ZDDP resulting in increased wear and corrosion.

International Publication WO 2005/087904 discloses a lubricant composition containing at least one hydroxycarboxylic acid ester or hydroxy polycarboxylic acid. The lubricant composition disclosed may also contain zinc dihydrocarbyldithiophosphates, or other phosphorous-containing additives such as trilauryl phosphate or triphenylphosphorothionate. The lubricant composition has anti-wear or anti-fatigue properties.

International Publication WO 2006/044411 discloses a low-sulphur, low-phosphorus, low-ash lubricant composition suitable for lubricating an internal combustion engine, containing a tartrate ester, or amide having 1 to 150 carbon atoms per ester of amide group.

US Patent 5,338,470 discloses alkylated citric acid derivatives obtained as a reaction product of citric acid and an alkyl alcohol or amine. The alkylated citric acid derivative is effective as an antiwear agent and friction modifier.

U.S. Patent 4,237,022 discloses tartrimides useful as additives in lubricants and fuels for effective reduction in squeal and friction as well as improvement in fuel economy.

U.S. Patent 4,952,328 discloses lubricating oil compositions for internal combustion engines, comprising (A) oil of lubricating viscosity, (B) a carboxylic derivative produced by reacting a succinic acylating agent with certain amines, and (C) a basic alkali metal salt of sulphonic or carboxylic acid.

U.S. Patent 4,326,972 discloses lubricant compositions for improving fuel economy of internal combustion engines. The composition includes a specific sulphurised composition (based on an ester of a carboxylic acid) and a basic alkali metal sulphonate.

U.S. Patent Application 60/867534 discloses malonate esters suitable as antiwear agents.

Canadian Patent CA 1 183 125 discloses lubricants for gasoline engines containing alkyl-ester tartrates, where the sum of carbon atoms on the alkyl groups is at least 8.

Consequently, it would be desirable to provide a lubricating composition capable of providing at least one of (i) reducing or preventing phosphorus emissions, (ii) reducing or preventing sulphur emissions, (ii) wholly or partially replacing ZDDP in lubricating oils, (iii) improving fuel economy, (iv) fuel economy retention/efficiency, and (v) lead and copper corrosion resistance. The present invention provides an antiwear agent capable of achieving at least one of (i), (ii) (iii), (iv), and (v). In addition it may also be desirable for the antiwear agent to not have a detrimental affect on other components of a mechanical device.

### SUMMERY OF THE INVENTION

In one embodiment the invention provides a lubricating composition comprising an oil of lubricating viscosity, an amine-containing friction modifier, and an ashless antiwear agent;
wherein the ashless antiwear agent is a diester derived from citric acid, the ashless antiwear agent is present at 0.05 to 10 wt% of the lubricating composition and the amine-containing friction modifier is present at 0.01 wt% to 5 wt% of the lubricating composition.

In one embodiment the lubricating composition is characterised as having at least one of (i) a sulphur content of 0.8 wt % or less, (ii) a phosphorus content of 0.2 wt % or less, or (iii) a sulphated ash content of 2 wt % or less.

In one embodiment the invention the lubricating composition is characterised as having (i) a sulphur content of 0.5 wt % or less, (ii) a phosphorus content of 0.1 wt % or less, and (iii) a sulphated ash content of 1.5 wt % or less.

In one embodiment the invention provides a method of lubricating an internal combustion engine comprising, supplying to the internal combustion engine a lubricating compositions as disclosed herein.

In one embodiment the invention provides for the use of a lubricating composition as disclosed herein for providing at least one of (i) reducing or preventing phosphorus emissions, (ii) reducing or preventing sulphur emissions, (ii) wholly or partially replacing ZDDP in lubricating oils, (iii) improving fuel economy, (iv) fuel economy retention/efficiency, and (v) lead and copper corrosion resistance.

### DETAILED DESCRIPTION OF THE INVENTION

The present invention provides a lubricating composition and a method for lubricating an engine as disclosed above.

### Amine-Containing Friction Modifier

The amine-containing friction modifier includes primary, secondary or tertiary amine. Typically the amine is hydrocarbyl- or hydroxyhydrocarbyl-substituted.

The amine-containing friction modifier may be a hydrocarbyl-substituted primary amine, a hydroxyhydrocarbyl- substituted amine, or mixtures thereof (or, in each instance, alkyl- or hydroxyalkyl-substituted amine). In one embodiment amine-containing friction modifier is a hydroxyhydrocarbyl-substituted amine, typically a tertiary amine.

When the amine-containing friction modifier is the hydroxybydrocarbyl- substituted amine and is a tertiary amine, the amine typically contains two hydroxybydrocarbyl groups and one hydrocarbyl group bonded directly to the nitrogen of the amine. The hydrocarbyl group may contain 1 to 30, or 4 to 26, or 12 to 20 carbon atoms. In one embodiment the hydrocarbyl group contains 16 to 18 carbon atoms.

In one embodiment the friction modifier may be a hydroxyhydrocarbyl- substituted (e.g., hydroxyalkyl-substituted) amine. The hydroxyhydrocarbyl- substituted amine may be derived from an alkoxy- group containing 1 to 10, 1 to 6 or 2 to 4 carbon atoms. Examples of a suitable alkoxylated amine (as such materials are often called) include ethoxylated amines. Ethoxylated amines may be derived from 1.79 % Ethomeen® T-12 and 0.90 % Tomah PA-1 as described in Example E of US Patent 5,703,023, column 28, lines 30 to 46. Other suitable alkoxylated amine compounds include commercial alkoxylated fatty amines known by the trademark "ETHOMEEN" and available from Akzo Nobel. Representative examples of these ETHOMEEN™ materials is ETHOMEEN™ C/12 (bis[2-hydroxyethyl]-cocoamine); ETHOMEEN™ C/20 (polyoxyethylene[10]cocoamine); ETHOMEEN™ S/12 (bis[2-hydroxyethyl]soyamine); ETHOMEEN™ T/12 (bis[2-hydroxyethyl]-tallow-amine); ETHOMEEN™ T/15 (polyoxyethylene-[5]tallowamine); ETHOMEEN™ 0/12 (bis[2-hydroxyethyl]oleyl-amine); ETHOMEEN™ 18/12 (bis[2-hydroxyethyl]octadecylamine); and ETHOMEEN™ 18/25 (polyoxyethylene[15]octadecylamine). Suitable fatty amines and ethoxylated fatty amines are also described in U.S. Patent 4,741,848.

When the hydrocarbyl- substituted amine is a primary amine, the hydrocarbyl group may contain 1 to 30, or 4 to 26, or 12 to 20 carbon atoms. In one embodiment the hydrocarbyl group contains 14 to 18 carbon atoms

Primary amines include ethylamine, propylamine, butylamine, 2-ethylhexylamine, octylamine, and dodecylamine, as well as such fatty amines as n-octylamine, n-decylamine, n-dodecylamine, n-tetradecylamine, n-hexadecylamine, n-octadecylamine and oleyamine. Other useful fatty amines include commercially available fatty amines such as "Armeen®" amines (products available from Akzo Chemicals, Chicago, Illinois), such as Armeen C, Armeen O, Armeen OL, Armeen T, Armeen HT, Armeen S and Armeen SD, wherein the letter designation relates to the fatty group, such as coco, oleyl, tallow, or stearyl groups.

The amine-containing friction modifier is present at 0.01 wt% to 5 wt%, and may be present at 0.02 wt % to 2 wt %, or 0.05 wt % to 1 wt % of the lubricating composition.

### Ashless Antiwear Agent

The ashless antiwear agent is a diester

Compositions intended for use in oils are typically oil-soluble and/or stably dispersible in an oil in which they are to be used. The term "oil-soluble" as used in this specification and appended claims does not necessarily mean that all the compositions in question are miscible or soluble in all proportions in all oils. Rather, it is intended to mean that the composition is soluble in an oil (mineral, synthetic, etc.) in which it is intended to function to an extent which permits the solution to exhibit one or more of the desired properties. Similarly, it is not necessary that such "solutions" be true solutions in the strict physical or chemical sense. They may instead be micro-emulsions or colloidal dispersions which, for the purpose of this invention, exhibit properties sufficiently close to those of true solutions to be, for practical purposes, interchangeable with them within the context of this invention.

The ashless antiwear agent includes a compound derived from a hydroxycarboxylic acid. The ashless antiwear agent is derived from at least one of hydroxy-polycarboxylic acid di-ester,
The ashless antiwear agent is a compound derived from citric acid.

US Patent Application 2005/198894 discloses suitable hydroxycarboxylic acid compounds, and methods of preparing the same.

Canadian Patent 1 183 125; US Patent Publication numbers 2006/0183647 and US-2006-0079413; US Patent Application number 60/867402; and British Patent 2 105 743 A, all disclose examples of suitable tartaric acid derivatives.

The ashless antiwear agent of the invention, may also function as rust and corrosion inhibitors, friction modifiers, antiwear agents and demulsifiers.

Examples of a suitable citric acid derivative include trialkyl citrates or borated trialkyl citrates. Suitable examples include triethyl citrate, tripentyl citrate with ethyl dipentyl citrate, borated triethyl citrate, tributyl citrate, triethyl citrate transesterified with 1,2-propandiol, triethyl O-acetyl citrate, triethyl citrate octadecyl succinate, oleyl citrate, or mixtures thereof. A more detailed description of suitable citrates is disclosed in WO 2005/087904 and U.S. Patent 5,338,470. Other suitable citrates include 2-ethylhexyl citrate, dodecyl citrate, or mixtures thereof.

In one embodiment the ashless antiwear agent is not borated.

The ashless antiwear agent is present at 0.05 to 10 wt%, and may be present at 0.1 to 5 wt % of the lubricating composition.

### Oils of Lubricating Viscosity

The lubricating composition comprises an oil of lubricating viscosity. Such oils include natural and synthetic oils, oil derived from hydrocracking, hydrogenation, and hydrofinishing, unrefined, refined and re-refined oils and mixtures thereof.

Unrefined oils are those obtained directly from a natural or synthetic source generally without (or with little) further purification treatment.

Refined oils are similar to the unrefined oils except they have been further treated in one or more purification steps to improve one or more properties. Purification techniques are known in the art and include solvent extraction, secondary distillation, acid or base extraction, filtration, percolation and the like.

Re-refined oils are also known as reclaimed or reprocessed oils, and are obtained by processes similar to those used to obtain refined oils and often are additionally processed by techniques directed to removal of spent additives and oil breakdown products.

Natural oils useful in making the inventive lubricants include animal oils, vegetable oils (e.g., castor oil,), mineral lubricating oils such as liquid petroleum oils and solvent-treated or acid-treated mineral lubricating oils of the paraffinic, naphthenic or mixed paraffinic-naphthenic types and oils derived from coal or shale or mixtures thereof.

Synthetic lubricating oils are useful and include hydrocarbon oils such as polymerized, oligomerised, or interpolymerised olefins (e.g., polybutylenes, polypropylenes, propyleneisobutylene copolymers); poly(1-hexenes), poly(1-octenes), trimers or oligomers of 1-decene, e.g., poly(1-decenes), such materials being often referred to as poly α-olefins, and mixtures thereof; alkyl-benzenes (e.g. dodecylbenzenes, tetradecylbenzenes, dinonylbenzenes, di-(2-ethylhexyl)-benzenes); polyphenyls (e.g., biphenyls, terphenyls, alkylated polyphenyls); diphenyl alkanes, alkylated diphenyl alkanes, alkylated diphenyl ethers and alkylated diphenyl sulphides and the derivatives, analogs and homologs thereof or mixtures thereof.

Other synthetic lubricating oils include polyol esters (such as Prolube®3970), diesters, liquid esters of phosphorus-containing acids (e.g., tricresyl phosphate, trioctyl phosphate, and the diethyl ester of decane phosphonic acid), or polymeric tetrahydrofurans. Synthetic oils may be produced by Fischer-Tropsch reactions and typically may be hydroisomerised Fischer-Tropsch hydrocarbons or waxes. In one embodiment oils may be prepared by a Fischer-Tropsch gas-to-liquid synthetic procedure as well as other gas-to-liquid oils.

Oils of lubricating viscosity may also be defined as specified in the American Petroleum Institute (API) Base Oil Interchangeability Guidelines. The five base oil groups are as follows: Group I (sulphur content >0.03 wt %, and/or <90 wt % saturates, viscosity index 80-120); Group II (sulphur content ≤0.03 wt %, and ≥90 wt % saturates, viscosity index 80-120); Group III (sulphur content ≤0.03 wt %, and ≥90 wt % saturates, viscosity index ≥120); Group IV (all polyalphaolefins (PAOs)); and Group V (all others not included in Groups I, II, III, or IV). The oil of lubricating viscosity comprises an API Group I, Group II, Group III, Group IV, Group V oil or mixtures thereof. Often the oil of lubricating viscosity is an API Group I, Group II, Group III, Group IV oil or mixtures thereof. Alternatively the oil of lubricating viscosity is often an API Group II, Group III or Group IV oil or mixtures thereof.

The amount of the oil of lubricating viscosity present is typically the balance remaining after subtracting from 100 wt % the sum of the amount of the ashless antiwear agent, the amine-containing friction modifier and the other performance additives.

The lubricating composition may be in the form of a concentrate and/or a fully formulated lubricant. If the lubricating composition of the invention (comprising (i) the ashless antiwear agent and (ii) the amine-containing friction modifier is in the form of a concentrate (which may be combined with additional oil to form, in whole or in part, a finished lubricant), the ratio of the of components of the invention to the oil of lubricating viscosity and/or to diluent oil include the ranges of 1:99 to 99:1 by weight, or 80:20 to 10:90 by weight.

### Other Performance Additives

The composition optionally comprises other performance additives. The other performance additives comprise at least one of metal deactivators, viscosity modifiers, detergents, friction modifiers (other than the ashless antiwear agent of the invention or the compound of formula (1)), antiwear agents (other than the ashless antiwear agent of the invention), corrosion inhibitors, dispersants, dispersant viscosity modifiers, extreme pressure agents, antioxidants, foam inhibitors, demulsifiers, pour point depressants, seal swelling agents and mixtures thereof. Typically, fully-formulated lubricating oil will contain one or more of these performance additives.

In one embodiment the lubricating composition comprises the ashless antiwear agent and further comprises at least one of a viscosity modifier, an antioxidant, an overbased detergent, a succinimide dispersant, or mixtures thereof.

In one embodiment the lubricating composition comprising the ashless antiwear agent further comprises a phosphorus-containing antiwear agent.

### Detergents

The lubricant composition optionally further comprises other known neutral or overbased detergents. Suitable detergent substrates include phenates, sulphur containing phenates, sulphonates, salixarates, salicylates, carboxylic acid, phosphorus acid, mono- and/or di- thiophosphoric acid, alkyl phenol, sulphur coupled alkyl phenol compounds, or saligenins. Various overbased detergents and their methods of preparation are described in greater detail in numerous patent publications, including WO2004/096957 and references cited therein. The detergent substrate is typically salted with a metal such as calcium, magnesium, potassium, sodium, or mixtures thereof. In one embodiment the lubricating composition further includes an overbased detergent. Typically the overbased detergent includes phenates, sulphur containing phenates, sulphonates, salixarates, salicylates, or mixtures thereof.

The detergent may be present at 0 wt % to 10 wt %, or 0.1 wt % to 8 wt %, or 1 wt % to 4 wt %, or greater than 4 to 8 wt %.

### Dispersants

Dispersants are often known as ashless-type dispersants because, prior to mixing in a lubricating oil composition, they do not contain ash-forming metals and they do not normally contribute any ash forming metals when added to a lubricant and polymeric dispersants. Ashless type dispersants are characterised by a polar group attached to a relatively high molecular weight hydrocarbon chain. Typical ashless dispersants include N-substituted long chain alkenyl succinimides. Examples of N-substituted long chain alkenyl succinimides include polyisobutylene succinimide with number average molecular weight of the polyisobutylene substituent in the range 350 to 5000, or 500 to 3000. Succinimide dispersants and their preparation are disclosed, for instance in US Patent 3,172,892 or US Patent 4,234,435 or in EP 0355895. Succinimide dispersants are typically the imide formed from a polyamine, typically a poly(ethyleneamine).

In one embodiment the invention further comprises at least one polyisobutylene succinimide dispersant derived from polyisobutylene with number average molecular weight in the range 350 to 5000, or 500 to 3000. The polyisobutylene succinimide may be used alone or in combination with other dispersants.

In one embodiment the invention further comprises at least one dispersant derived from polyisobutylene succinic anhydride, an amine and zinc oxide to form a polyisobutylene succinimide complex with zinc. The polyisobutylene succinimide complex with zinc may be used alone or in combination.

Another class of ashless dispersant is Mannich bases. Mannich dispersants are the reaction products of alkyl phenols with aldehydes (especially formaldehyde) and amines (especially polyalkylene polyamines). The alkyl group typically contains at least 30 carbon atoms.

The dispersants may also be post-treated by conventional methods by a reaction with any of a variety of agents. Among these are boron, urea, thiourea, dimercaptothiadiazoles, carbon disulphide, aldehydes, ketones, carboxylic acids, hydrocarbon-substituted succinic anhydrides, maleic anhydride, nitriles, epoxides, and phosphorus compounds.

The dispersant may be present at 0 wt % to 20 wt %, or 0.1 wt % to 15 wt%, or 0.1 wt % to 10 wt %, or 1 wt% to 6 wt %, or 7 wt % to 12wt % of the lubricating composition.

### Antioxidants

Antioxidant compounds are known and include for example, sulphurised olefins (typically sulphurised 4-carbobutoxy cyclohexene, or triphenylphosphite equivalents thereof, or olefin sulphide), alkylated diphenylamines (e.g., nonyl diphenylamine, di-nonyl diphenylamine, octyl diphenylamine, di-octyl diphenylamine), hindered phenols, oil-soluble molybdenum compounds, or mixtures thereof. Antioxidant compounds may be used alone or in combination. The antioxidant may be present in ranges 0 wt % to 20 wt %, or 0.1 wt % to 10 wt %, or 1 wt % to 5 wt %, of the lubricating composition.

The hindered phenol antioxidant often contains a secondary butyl and/or a tertiary butyl group as a sterically hindering group. The phenol group is often further substituted with a hydrocarbyl group and/or a bridging group linking to a second aromatic group. Examples of suitable hindered phenol antioxidants include 2,6-di-tert-butylphenol, 4-methyl-2,6-di-tert-butylphenol, 4-ethyl-2,6-di-tert-butylphenol, 4-propyl-2,6-di-tert-butylphenol or 4-butyl-2,6-di-tert-butylphenol, or 4-dodecyl-2,6-di-tert-butylphenol. In one embodiment the hindered phenol antioxidant is an ester and may include, e.g., Irganox™ L-135 from Ciba or an addition product derived from 2,6-di-tert-butylphenol and an alkyl acrylate, wherein the alkyl group may contain 1 to 18, or 2 to 12, or 2 to 8, or 2 to 6, or 4 carbon atoms. A more detailed description of suitable ester-containing hindered phenol antioxidant chemistry is found in US Patent 6,559,105.

The oil-soluble molybdenum compound may have the functional performance of an antiwear agent, an antioxidant, a friction modifier, or mixtures thereof. Typically, the oil-soluble molybdenum compound includes molybdenum dithiocarbamates, molybdenum dialkyldithiophosphates, amine salts of molybdenum compounds, molybdenum xanthates, molybdenum sulphides, molybdenum carboxylates, molybdenum alkoxides, or mixtures thereof. The molybdenum sulphides include molybdenum disulphide. The molybdenum disulphide may be in the form of stable dispersions. In one embodiment the oil-soluble molybdenum compound may be selected from the group consisting of molybdenum dithiocarbamates, molybdenum dialkyldithiophosphates, amine salts of molybdenum compounds, and mixtures thereof. In one embodiment the oil-soluble molybdenum compound is a molybdenum dithiocarbamate.

Suitable examples of molybdenum dithiocarbamates which may be used as an antioxidant include commercial materials sold under the trade names such as Molyvan 822™ and Molyvan™ A from R. T. Vanderbilt Co., Ltd., and Adeka Sakura-Lube™ S-100, S-165, S-515, and S-600 from Asahi Denka Kogyo K. K and mixtures thereof.

The oil-soluble molybdenum compound may be present in an amount sufficient to provide 0.5 ppm to 2000 ppm, 1 ppm to 700 ppm, 1 ppm to 550 ppm, 5 ppm to 300 ppm, or 20 ppm to 250 ppm of molybdenum.

### Viscosity Modifiers

Viscosity modifiers include hydrogenated copolymers of styrenebutadiene, ethylene-propylene copolymers, polyisobutenes, hydrogenated styrene-isoprene polymers, hydrogenated isoprene polymers, polymethacrylates, polyacrylates, polyalkyl styrenes, hydrogenated alkenyl aryl conjugated diene copolymers, polyolefins, esters of maleic anhydride-styrene copolymers, or esters of (alpha-olefin maleic anhydride) copolymers, or mixtures thereof.

### Dispersant Viscosity Modifiers

Dispersant viscosity modifiers (often referred to as DVM), include functionalised polyolefins, for example, ethylene-propylene copolymers that have been functionalised with the reaction product of an acylating agent (such as maleic anhydride) and an amine; polymethacrylates functionalised with an amine, or esterified maleic anhydride-styrene copolymers reacted with an amine.

The total amount of viscosity modifier and/or dispersant viscosity modifier may be 0 wt % to 20 wt %, 0.1 wt % to 15 wt %, or 0.1 wt % to 10 wt %, of the lubricating composition.

### Antiwear Agents

The lubricant composition optionally further comprises at least one other antiwear agent other than the ashless antiwear agent of the invention. Examples of suitable antiwear agents include phosphate esters, sulphurised olefins, sulphur-containing anti-wear additives including metal dihydrocarbyldithiophosphates (such as zinc dialkyldithiophosphates), thiocarbamate-containing compounds including, thiocarbamate esters, alkylene-coupled thiocarbamates, and bis(S-alkyldithiocarbamyl) disulphides.

The dithiocarbamate-containing compounds may be prepared by reacting a dithiocarbamate acid or salt with an unsaturated compound. The dithiocarbamate containing compounds may also be prepared by simultaneously reacting an amine, carbon disulphide and an unsaturated compound. Generally, the reaction occurs at a temperature of 25 °C to 125 °C. US Patents 4,758,362 and 4,997,969 describe dithiocarbamate compounds and methods of making them.

Examples of suitable olefins that may be sulphurised to form an the sulphurised olefin include propylene, butylene, isobutylene, pentene, hexane, heptene, octane, nonene, decene, undecene, dodecene, undecyl, tridecene, tetradecene, pentadecene, hexadecene, heptadecene, octadecene, octadecenene, nonodecene, eicosene or mixtures thereof. In one embodiment, hexadecene, heptadecene, octadecene, octadecenene, nonodecene, eicosene or mixtures thereof and their dimers, trimers and tetramers are especially useful olefins. Alternatively, the olefin may be a Diels-Alder adduct of a diene such as 1,3-butadiene and an unsaturated ester, such as, butylacrylate.

Another class of sulphurised olefin includes fatty acids and their esters. The fatty acids are often obtained from vegetable oil or animal oil and typically contain 4 to 22 carbon atoms. Examples of suitable fatty acids and their esters include triglycerides, oleic acid, linoleic acid, palmitoleic acid or mixtures thereof. Often, the fatty acids are obtained from lard oil, tall oil, peanut oil, soybean oil, cottonseed oil, sunflower seed oil or mixtures thereof. In one embodiment fatty acids and/or ester are mixed with olefins, such as α-olefins.

In one embodiment the composition further comprises a monoester of a polyol and an aliphatic carboxylic acid, often an acid containing 12 to 24 carbon atoms. Often the monoester of a polyol and an aliphatic carboxylic acid is in the form of a mixture with a sunflower oil or the like, which may be present in the ashless antiwear agent mixture include 5 to 95, or in other embodiments 10 to 90, or 20 to 85, or 20 to 80 weight percent of said mixture. The aliphatic carboxylic acids (especially a monocarboxylic acid) which form the esters are those acids typically containing 12 to 24 or 14 to 20 carbon atoms. Examples of carboxylic acids include dodecanoic acid, stearic acid, lauric acid, behenic acid, and oleic acid.

Polyols include diols, triols, and alcohols with higher numbers of alcoholic OH groups. Polyhydric alcohols include ethylene glycols, including di-, tri- and tetraethylene glycols; propylene glycols, including di-, tri- and tetrapropylene glycols; glycerol; butanediol; hexanediol; sorbitol; arabitol; mannitol; sucrose; fructose; glucose; cyclohexane diol; erythritol; and pentaerythritols, including di- and tripentaerythritol. Often the polyol is diethylene glycol, triethylene glycol, glycerol, sorbitol, pentaerythritol or dipentaerythritol. The commercial material known as glycerol monooleate is believed to include about 60 ± 5 percent by weight of the chemical species "glycerol monooleate," along with 35 ± 5 percent glycerol dioleate, and less than about 5 percent trioleate and oleic acid. The amounts of the monoesters, described below, are the amounts of the commercial grade material.

In one embodiment the composition further comprises an ashless antiwear agent (other than the compound of Formula (1), which may also be described as a friction modifier) may be a fatty acid amide (such as oleyl amide).

The antiwear agent may be present in ranges including 0 wt % to 15 wt %, or 0 wt % to 10 wt %, or 0.05 wt % to 5 wt %, or 0.1 wt % to 3 wt % of the lubricating composition.

In one embodiment the lubricating composition is free of zinc dihydrocarbyl dithiophosphate. In one embodiment the lubricating composition further includes zinc dihydrocarbyl dithiophosphate.

### Extreme Pressure Agents

Extreme Pressure (EP) agents that are soluble in the oil include sulphur- and chlorosulphur-containing EP agents, chlorinated hydrocarbon EP agents and phosphorus EP agents. Examples of such EP agents include chlorinated wax; organic sulphides and polysulphides such as dibenzyldisulphide, bis-(chlorobenzyl) disulphide, dibutyl tetrasulphide, sulphurised methyl ester of oleic acid, sulphurised alkylphenol, sulphurised dipentene, sulphurised terpene, and sulphurised Diels-Alder adducts; phosphosulphurised hydrocarbons such as the reaction product of phosphorus sulphide with turpentine or methyl oleate; phosphorus esters such as the dihydrocarbon and trihydrocarbon phosphites, e.g., dibutyl phosphite, diheptyl phosphite, dicyclohexyl phosphite, pentylphenyl phosphite; dipentylphenyl phosphite, tridecyl phosphite, distearyl phosphite and polypropylene substituted phenyl phosphite; metal thiocarbamates such as zinc dioctyldithiocarbamate and barium heptylphenol diacid; amine salts of alkyl and dialkylphosphoric acids, including, for example, the amine salt of the reaction product of a dialkyldithiophosphoric acid with propylene oxide; and mixtures thereof.

### Friction Modifiers

In one embodiment the composition further comprises a friction modifier other than the amine-containing friction modifier of the invention. Typically the friction modifier may be present in ranges including 0 wt % to 10 wt %, or 0 wt % to 8 wt %, or 0 wt % to 4 wt %.

Friction modifiers may also encompass materials such as sulphurised fatty compounds and olefins, sunflower oil or monoester of a polyol and an aliphatic carboxylic acid (all these friction modifiers have been described as antioxidants or antiwear agents).

In one embodiment the friction modifier is a long chain fatty acid ester (previously described above as an ashless antiwear agent). In another embodiment the long chain fatty acid ester is a mono-ester and in another embodiment the long chain fatty acid ester is a (tri)glyceride. In one embodiment the friction modifier is a long chain fatty amide, a long chain fatty ester, a long chain fatty epoxide derivatives, or a long chain fatty imidazoline.

### Other Additives

Other performance additives such as corrosion inhibitors include those described in paragraphs 5 to 8 of US Application US05/038319 (filed on October 25, 2004 McAtee and Boyer as named inventors), octylamine octanoate, and condensation products of dodecenyl succinic acid or anhydride and a fatty acid such as oleic acid with a polyamine. In one embodiment the corrosion inhibitors include the Synalox® corrosion inhibitor. The Synalox® corrosion inhibitor is typically a homopolymer or copolymer of propylene oxide. The Synalox® corrosion inhibitor is described in more detail in a product brochure with Form No. 118-01453-0702 AMS, published by The Dow Chemical Company. The product brochure is entitled "SYNALOX Lubricants, High-Performance Polyglycols for Demanding Applications."

Metal deactivators including derivatives of benzotriazoles (typically tolyltriazole), dimercaptothiadiazole derivatives, 1,2,4-triazoles, benzimidazoles, 2-alkyldithiobenzimidazoles, or 2-alkyldithiobenzothiazoles; foam inhibitors including copolymers of ethyl acrylate and 2-ethylhexylacrylate and optionally vinyl acetate; demulsifiers including trialkyl phosphates, polyethylene glycols, polyethylene oxides, polypropylene oxides and (ethylene oxide-propylene oxide) polymers; pour point depressants including esters of maleic anhydride-styrene, polymethacrylates, polyacrylates or polyacrylamides.

### Industrial Application

The lubricating composition may be utilised in a range of surfaces typically found in mechanical devices, including aluminium-alloy surfaces. The mechanical devices include an internal combustion engine, a gearbox, an automatic transmission, a hydraulic or a turbine. Typically the lubricating composition may be an engine oil, a gear oil, an automatic transmission oil, a hydraulic fluid, a turbine oil, a metal working fluid or a circulating oil. In one embodiment the mechanical device is an internal combustion engine.

In one embodiment the internal combustion engine may be a diesel fuelled engine, a gasoline fuelled engine, a natural gas fuelled engine or a mixed gasoline/alcohol fuelled engine. In one embodiment the internal combustion engine may be a diesel fuelled engine and in another embodiment a gasoline fuelled engine.

The internal combustion engine may be a 2-stroke or 4-stroke engine. Suitable internal combustion engines include marine diesel engines, aviation piston engines, low-load diesel engines, and automobile and truck engines.

In one embodiment the internal combustion engine contains components of an aluminium-alloy. The aluminium-alloy includes aluminium silicates, aluminium oxides, or other ceramic materials. In one embodiment the aluminium-alloy is an aluminium-silicate surface. As used herein, the term "aluminium alloy" is intended to be synonymous with "aluminium composite" and to describe a component or surface comprising aluminium and another component intermixed or reacted on a microscopic or nearly microscopic level, regardless of the detailed structure thereof. This would include any conventional alloys with metals other than aluminium as well as composite or alloy-like structures with non-metallic elements or compounds such as with ceramic-like materials.

The lubricant composition for an internal combustion engine may be suitable for any engine lubricant irrespective of the sulphur, phosphorus or sulphated ash (ASTM D-874) content. The sulphur content of the engine oil lubricant may be 1 wt % or less, or 0.8 wt % or less, or 0.5 wt % or less, or 0.3 wt % or less. In one embodiment the sulphur content may be in the range of 0.001 wt % to 0.5 wt %, or 0.01 wt % to 0.3 wt %. The phosphorus content may be 0.2 wt % or less, or 0.1 wt % or less, or 0.085 wt % or less, or even 0.06 wt % or less, 0.055 wt % or less, or 0.05 wt % or less. In one embodiment the phosphorus content may be 100 ppm to 1000 ppm, or 325 ppm to 700 ppm. The total sulphated ash content may be 2 wt % or less, or 1.5 wt % or less, or 1.1 wt % or less, or 1 wt % or less, or 0.8 wt % or less, or 0.5 wt % or less. In one embodiment the sulphated ash content may be 0.05 wt % to 0.9 wt %, or 0.1 wt % or 0.2 wt % to 0.45 wt %. In another embodiment the sulphur content is 0.4 wt % or less, the phosphorus content is 0.08 wt % or less, and the sulphated ash is 1 wt % or less. In yet another embodiment the sulphur content is 0.3 wt% or less, the phosphorus content is 0.05 wt % or less, and the sulphated ash is 0.8 wt % or less.

In one embodiment the lubricating composition is an engine oil, wherein the lubricating composition is characterised as having (i) a sulphur content of 0.5 wt % or less, (ii) a phosphorus content of 0.1 wt % or less, and (iii) a sulphated ash content of 1.5 wt % or less.

In one embodiment the lubricating composition is suitable for a 2-stroke or a 4-stroke marine diesel internal combustion engine. In one embodiment the marine diesel combustion engine is a 2-stroke engine. The ashless antiwear agent of the invention may be added to a marine diesel lubricating composition at 0.01 to 20 wt %, or 0.05 to 10 wt %, or 0.1 to 5 wt %.

The following examples provide illustrations of the invention. These examples are non-exhaustive and are not intended to limit the scope of the invention.

### EXAMPLES (Not according to the invention)

As used herein all of the quantities for dispersants, detergents and viscosity modifiers shown below include conventional amount of diluent oil Typically the diluent oil constitutes 20 wt % to 90 wt % of each component. For antiwear agents, corrosion inhibitors, antioxidants the amounts shown are on an actives basis i.e. excluding diluent oil because the components are typically not carried in diluent oil.

Example 1 (EX1) (Not according to the invention): A lubricating composition is prepared containing 0.2 wt % of di-2-ethylhexyl tartrate, 0.2 wt % of hydroxyalkyl amine (Ethomeen T/12), 0.86 wt % of other antiwear agents (including zinc dialkdithiophosphate), 5 wt % of dispersants, 1.5 wt % of detergents, 1.3 wt % of antioxidants, 4.3 wt % of viscosity modifier. The lubricating composition has a phosphorus content of about 760 ppm, and a sulphur content of 0.25 wt %.

Comparative Example 1 (CE1): is similar to Example 2 except the composition does not contain di-2-ethylhexyl tartrate and does not contain hydroxylalkyl amine.

Comparative Example 2 (CE2): is similar to Example 2 except the composition does not contain hydroxyalkyl amine.

Comparative Example 3 (CE3): is similar to Example 2 except the composition does not contain di-2-ethylhexyl tartrate.

Test 1: 10 g samples of the examples above are each treated with one volume percent of cumene hydroperoxide. The samples (2 ml portions) are then evaluated for wear performance in an isothermal temperature high frequency reciprocating rig (HFRR) available from PCS Instruments. HFRR conditions for the evaluations are 500g load, 75 minute duration, 1000 micrometer stroke, 20 hertz frequency, and at 105 °C. Wear scar in micrometers, coefficient of friction and film formation as percent film thickness are then measured with lower wear scar values and higher film formation values indicating improved wear performance. Typically, an engine oil lubricant with a coefficient of friction of less than 0.18 is acceptable. All of the samples evaluated have acceptable wear scar performance.

Test 2: ASTM D6594-05 testing diesel engine lubricants to determine their tendency to corrode various metals, specifically alloys of lead and copper commonly used in cam followers and bearings. The pass levels for copper and lead corrosion are less than 20 ppm and less than 100 ppm respectively.

Test 3: Cold crank simulator at -30 °C (CCS -30), as specified by ASTM D5293-04. Typically better results are obtained for samples with a lower Centipoise indicate better performance.

The results obtained for the three tests are:

| | | Example | | | |
|---|---|---|---|---|---|
| Test | Parameter Evaluated | CE1 | CE2 | CE3 | EX1 |
| Test 1: HFRR Data | % Film Formation | 0 | 0 | 97 | 72 |
| | Coefficient of Friction | 0.199 | 0.163 | 0.135 | 0.154 |
| Test 2: ASTM D6594-05 | Copper (ppm) | 73 | 8 | 88 | 11 |
| | Lead (ppm) | 3 | 363 | 8 | 40 |
| Test 3: CCS -30 °C | Viscosity (Centipoise) | 4344 | 4469 | 4407 | 4173 |

The results obtained for CE1 indicate poor cold crank performance at - 30 °C, show significant copper corrosion, and a coefficient of friction that is too high. CE2 has high lead corrosion and poor cold crank performance at -30 °C. CE3 has high copper corrosion and poor cold crank performance at -30 °C. Thus lubricating compositions based on CE1, CE2 and CE3 would provide poor performance in an internal combustion engine. In contrast, the results obtained for the lubricating composition EX1 demonstrate acceptable performance in all of the parameters evaluated above. The lubricating composition of the invention is capable of at least one of, (most or all of) (i) reducing or preventing phosphorus emissions, (ii) reducing or preventing sulphur emissions, (ii) wholly or partially replacing ZDDP in lubricating oils, (iii) improving fuel economy, (iv) fuel economy retention/efficiency, and (v) lead and copper corrosion resistance.

It is known that some of the materials described above may interact in the final formulation, so that the components of the final formulation may be different from those that are initially added. The products formed thereby, including the products formed upon employing lubricant composition of the present invention in its intended use, may not be susceptible of easy description. Nevertheless, all such modifications and reaction products are included within the scope of the present invention; the present invention encompasses lubricant composition prepared by admixing the components described above.

Unless otherwise indicated, each chemical or composition referred to herein should be interpreted as being a commercial grade material which may contain the isomers, by-products, derivatives, and other such materials which are normally understood to be present in the commercial grade. However, the amount of each chemical component is presented exclusive of any solvent or diluent oil, which may be customarily present in the commercial material, unless otherwise indicated. It is to be understood that the upper and lower amount, range, and ratio limits set forth herein may be independently combined. Similarly, the ranges and amounts for each element of the invention may be used together with ranges or amounts for any of the other elements.

As used herein, the term "hydrocarbyl substituent" or "hydrocarbyl group" is used in its ordinary sense, which is well-known to those skilled in the art. Specifically, it refers to a group having a carbon atom directly attached to the remainder of the molecule and having predominantly hydrocarbon character. Examples of hydrocarbyl groups include:
(i) hydrocarbon substituents, that is, aliphatic (e.g., alkyl or alkenyl), alicyclic (e.g., cycloalkyl, cycloalkenyl) substituents, and aromatic-, aliphatic-, and alicyclic-substituted aromatic substituents, as well as cyclic substituents wherein the ring is completed through another portion of the molecule (e.g., two substituents together form a ring);
(ii) substituted hydrocarbon substituents, that is, substituents containing non-hydrocarbon groups which, in the context of this invention, do not alter the predominantly hydrocarbon nature of the substituent (e.g., halo (especially chloro and fluoro), hydroxy, alkoxy, mercapto, alkylmercapto, nitro, nitroso, and sulphoxy);
(iii) hetero substituents, that is, substituents which, while having a predominantly hydrocarbon character, in the context of this invention, contain other than carbon in a ring or chain otherwise composed of carbon atoms. Heteroatoms include sulphur, oxygen, nitrogen, and encompass substituents as pyridyl, furyl, thienyl and imidazolyl. In general, no more than two, preferably no more than one, non-hydrocarbon substituent will be present for every ten carbon atoms in the hydrocarbyl group; typically, there will be no non-hydrocarbon substituents in the hydrocarbyl group.

As will be evident, the antiwear agent described herein may be an oil-soluble derivative of a molecule containing a first carboxy group and at least one additional -OH, -NHR, or =O moiety separated from the carbon of said first carboxy group by a chain of 2 or 3 atoms, where R is hydrogen or alkyl, e.g, C1-6 alkyl.

## Claims

1. A lubricating composition comprising an oil of lubricating viscosity, an amine-containing friction modifier, and an ashless antiwear agent;
wherein the ashless antiwear agent is a diester derived from citric acid, the ashless antiwear agent is present at 0.05 to 10 wt% of the lubricating composition and the amine-containing friction modifier is present at 0.01 wt% to 5 wt% of the lubricating composition.

2. The lubricating composition of claim 1, wherein the ashless antiwear agent is present at 0.1 to 5 wt % of the lubricating composition.

3. The lubricating composition of claim 1, wherein the amine-containing friction modifier is a primary or secondary hydrocarbyl amine, a hydroxyalkyl amine, or mixtures thereof.

4. The lubricating composition of claim 3, wherein the amine-containing friction modifier is a hydroxyalkyl amine.

5. The lubricating composition of claim 1, wherein the amine-containing friction modifier is a tertiary amines.

6. The lubricating composition of claim 1, wherein the amine-containing friction modifier is present at 0.02 wt % to 2 wt % or 0.05 wt % to 1 wt % of the lubricating composition

7. The lubricating compositions of claim 1, wherein the lubricating composition is characterised as having (i) a sulphur content of 0.5 wt % or less, (ii) a phosphorus content of 0.1 wt % or less, and (iii) a sulphated ash content of 1.5 wt % or less.

8. The lubricating composition of claim 1 further comprises at least one of a viscosity modifier, an antioxidant, an overbased detergent, a succinimide dispersant, or mixtures thereof.

9. The lubricating composition of claim 1 further comprising an overbased detergent, wherein the overbased detergent is selected from the group consisting of non-sulphur-containing phenates, sulphur-containing phenates, sulphonates, salixarates, salicylates, and mixtures thereof.

10. A method of lubricating an internal combustion engine comprising, supplying to the internal combustion engine the lubricating composition of claim 1.

## Patentansprüche

1. Schmierende Zusammensetzung, umfassend ein Öl mit schmierender Viskosität, einen Amin-enthaltenden Reibungsmodifizierer und ein aschefreies Antiverschleißmittel, wobei das aschefreie Antiverschleißmittel ein Diester ist, der von Zitronensäure abgeleitet ist, wobei das aschefreie Antiverschleißmittel mit 0,05 bis 10 Gew.-% der schmierenden Zusammensetzung vorliegt, und wobei der Amin-enthaltende Reibungsmodifizierer mit 0,01 Gew.-% bis 5 Gew.-% der schmierenden Zusammensetzung vorliegt.

2. Schmierende Zusammensetzung nach Anspruch 1, wobei das aschefreie Antiverschleißmittel mit 0,1 bis 5 Gew.-% der schmierenden Zusammensetzung vorliegt.

3. Schmierende Zusammensetzung nach Anspruch 1, wobei der Amin-enthaltende Reibungsmodifizierer ein primäres oder sekundäres Kohlenwasserstoff-Amin, ein Hydroxyalkylamin oder Gemische davon ist.

4. Schmierende Zusammensetzung nach Anspruch 3, wobei der Amin-enthaltende Reibungsmodifizierer ein Hydroxyalkylamin ist.

5. Schmierende Zusammensetzung nach Anspruch 1, wobei der Amin-enthaltende Reibungsmodifizierer ein tertiäres Amin ist.

6. Schmierende Zusammensetzung nach Anspruch 1, wobei der Amin-enthaltende Reibungsmodifizierer mit 0,02 Gew.-% bis 2 Gew.-% oder 0,05 Gew.-% bis 1 Gew.-% der schmierenden Zusammensetzung vorliegt.

7. Schmierende Zusammensetzung nach Anspruch 1, wobei die schmierende Zusammensetzung **gekennzeichnet ist durch** (i) einen Schwefelgehalt von 0,5 Gew.-% oder weniger, (ii) einen Phosphorgehalt von 0,1 Gew.-% oder weniger und (iii) einen Sulfataschegehalt von 1,5 Gew.-% oder weniger.

8. Schmierende Zusammensetzung nach Anspruch 1, welche weiterhin wenigstens eines unter einem Viskositätsmodifizierer, einem Antioxidationsmittel, einem überbasischen Detergenz, einem Bersteinimid-Dispergiermittel oder Gemische davon umfasst.

9. Schmierende Zusammensetzung nach Anspruch 1, welche weiterhin ein überbasisches Detergenz umfasst, wobei das überbasische Detergenz aus der Gruppe ausgewählt ist, bestehend aus nicht-schwefelhaltigen Phenaten, schwefelhaltigen Phenaten, Sulfonaten, Salixaraten, Salicylaten und Gemischen davon.

10. Verfahren zum Schmieren eines Verbrennungsmotors, bei dem man dem Verbrennungsmotor die schmierende Zusammensetzung nach Anspruch 1 zuführt.

## Revendications

1. Composition lubrifiante comprenant une huile de viscosité lubrifiante, un modificateur de frottement contenant une ou des amines et un agent anti-usure sans cendres ;
où l'agent anti-usure sans cendre est un diester dérivé de l'acide citrique, l'agent anti-usure sans cendre est présent à raison de 0,05 à 10 % en poids de la composition lubrifiante et le modificateur de frottement contenant une ou des amines est présent à raison de 0,01 % en poids à 5 % en poids de la composition lubrifiante.

2. Composition lubrifiante selon la revendication 1 où l'agent anti-usure sans cendre est présent à raison de 0,1 à 5 % en poids de la composition lubrifiante.

3. Composition lubrifiante selon la revendication 1 où le modificateur de frottement contenant une ou des amines est une hydrocarbylamine primaire ou secondaire, une hydroxyalkylamine ou des mélanges de celles-ci.

4. Composition lubrifiante selon la revendication 1 où le modificateur de frottement contenant une ou des amines est une hydroxyalkylamine.

5. Composition lubrifiante selon la revendication 1 où le modificateur de frottement contenant une ou des amines est une amine tertiaire.

6. Composition lubrifiante selon la revendication 1 où le modificateur de frottement contenant une ou des amines est présent à raison de 0,02 % en poids à 2 % en poids ou à raison de 0,05 % en poids à 1 % en poids de la composition lubrifiante.

7. Composition lubrifiante selon la revendication 1 où la composition lubrifiante est **caractérisée en ce qu'**elle a (i) une teneur en soufre de 0,5 % en poids ou moins, (ii) une teneur en phosphore de 0,1 % en poids ou moins et (iii) une teneur en cendres sulfatées de 1,5 % en poids ou moins.

8. Composition lubrifiante selon la revendication 1 comprend en outre au moins l'un d'un modificateur de viscosité, un antioxydant, un détergent surbasé, un dispersant succinimide ou des mélanges de ceux-ci.

9. Composition lubrifiante selon la revendication 1 comprenant en outre un détergent surbasé, où le détergent surbasé est choisi dans le groupe consistant en les phénates ne contenant pas de soufre, les phénates contenant du soufre, les sulfonates, les salixarates, les salicylates et leurs mélanges.

10. Procédé de lubrification d'un moteur à combustion interne comprenant l'apport au moteur à combustion interne de la composition lubrifiante selon la revendication 1.
